

## UNITED STATES PATENT OFFICE

JULIUS C. FUNCKE, OF ELIZABETHTON, TENNESSEE, ASSIGNOR TO AMERICAN GLANZSTOFF CORPORATION, OF NEW YORK, N. Y., A CORPORATION OF DELAWARE

## DESULPHURIZATION

No Drawing.

Application filed September 1, 1931. Serial No. 560,667.

My new invention has to do with a novel and advantageous method for desulphurizing artificial filaments formed by the viscose process.

5 One object of my invention is to eliminate carbon disulphide.

Another object is to present a process which facilitates the desulphurization of artificial filaments of viscose.

10 Other objects will readily become apparent from a reading of the following specification.

In the manufacture of artificial filaments, films, etc. from viscose, the cellulose is treated with a caustic solution, and then with carbon bisulphide in order to form a xanthate. This xanthate, in solution, forms viscose. Viscose is extruded, for example, to form filaments, which must be deacidified, bleached, desulphurized, etc. The present invention has to do with a novel method for use in this desulphurization step.

Usually there is a deposit of about 1% of a sulphur on the filaments, giving them a 25 yellowish-gray color. As a desulphurizing means ammonium sulphide may be used. The ammonium sulphide solution acts to dissolve the sulphur, forming ammonium polysulphide.

30 It has been found that some carbon bisulphide is also retained by the filaments, and I have devised a method whereby this carbon bisulphide may be eliminated. Certain difficulties arise through the presence of 35 the carbon bisulphide, and it has been found that the desulphurizing agent used is weakened through the formation of trithiocarbonates from the action of the carbon bisulphide therewith.

40 I have discovered that if an amine is added to the desulphurizing solution the desulphurization is facilitated and the carbon bisulphide removed, because the amine, acting as a catalyst, combines therewith. Afterwards the compound breaks down to form the original amine plus some sulphides.

I have found that primary amines (such 45 as methylamine  $\text{CH}_3\text{NH}_2$ ); secondary amines (such as dimethylamine  $\text{NH}(\text{CH}_3)_2$ );

or tertiary amines (such as trimethylamine  $\text{N}(\text{CH}_3)_3$ ), may be used.

One example of my method follows:

To the desulphurizing solution I add an amine, here aniline, in a proportion of one 55 gram of aniline to one liter of the desulphurizing solution. This solution, here in this example, contains from 10 to 20 grams of ammonium or sodium sulphide per liter. The reactions which take place are as follows:



65 These equations indicate the manner in which an amine, added as a catalyst, removes the carbon bisulphide, which is detrimental in its action, by converting it into either ammonium or sodium sulphide. This 70 ammonium or sodium sulphide. This ammonium or sodium sulphide may later be reused.

75 Although I have used aniline as an example, it must be understood that I do not limit myself thereto, and wish to be limited only by the scope of the claims presented.

Having fully set forth my invention as required by the patent statutes, what I desire to claim is:

80 1. In the step of desulphurizing artificial cellulosic products formed from viscose, the step of adding an amine to the desulphurizing medium used.

85 2. In a process of the class described, the step of adding to a desulphurizing medium an organic amine that acts as a catalyst.

3. As a desulphurizing solution, a solution of sodium sulphide, water, and amine.

90 4. In a process of the class described, the step of desulphurizing a viscose yarn in a solution comprising:

|                   | Percent by weight |
|-------------------|-------------------|
| Ammonium sulphide | 10-20 95          |
| Aniline           | 1                 |

in water to make up a liter of solution.

95 5. In the step of desulphurizing artificial cellulosic products from viscose, the step of 100

adding a catalyst consisting of an amine to the desulphurizing medium used.

6. As a desulphurizing agent, a solution of ammonium sulphide, water, and an amine.

5 7. As a desulphurizing medium a solution containing a sulphide of the group consisting of sodium and ammonium, water, and an amine.

8. As a desulphurizing medium, a solution 10 comprising a sulphide of the group consisting of sodium and ammonium, water, and aniline.

In testimony whereof I affix my signature.

JULIUS C. FUNCKE.

15

20

25

30

35

40

45

50

55

60

65